

|      |                                                                                                                           |                                                                                                               |           |                            |                    |
|------|---------------------------------------------------------------------------------------------------------------------------|---------------------------------------------------------------------------------------------------------------|-----------|----------------------------|--------------------|
| [72] | Inventors                                                                                                                 | E. Scudder Mackey<br>Binghamton, N.Y.;<br>Fritz Dersch, Binghamton, N.Y.; Fred S.<br>Eiseman, Maplewood, N.J. | [50]      | Field of Search.....       | 96/107,<br>109, 87 |
| [21] | Appl. No.                                                                                                                 | 697,323                                                                                                       | [56]      | References Cited           |                    |
| [22] | Filed                                                                                                                     | Jan. 12, 1968                                                                                                 |           | UNITED STATES PATENTS      |                    |
| [45] | Patented                                                                                                                  | Oct. 26, 1971                                                                                                 | 3,255,013 | 6/1966 Dersch et al.....   | 96/107             |
| [73] | Assignee                                                                                                                  | GAF Corporation<br>New York, N.Y.                                                                             |           | FOREIGN PATENTS            |                    |
|      |                                                                                                                           |                                                                                                               | 1,015,023 | 12/1965 Great Britain..... | 96/107             |
| [54] | <b>PHOTOGRAPHIC ELEMENT CONTAINING A<br/>PHOSPHORIC ACID ESTER OF A BUTYNEDIOL-<br/>ALKYLENE</b><br>9 Claims, No Drawings |                                                                                                               |           |                            |                    |
| [52] | U.S. Cl.                                                                                                                  | 96/107,<br>96/109                                                                                             |           |                            |                    |
| [51] | Int. Cl.                                                                                                                  | G03c 1/28,<br>G03c 1/34                                                                                       |           |                            |                    |

*Primary Examiner*—Norman G. Torchin  
*Assistant Examiner*—Richard E. Fichter  
*Attorneys*—George L. Tone and Walter G. Hensel

**ABSTRACT:** A photographic element having incorporated in the light-sensitive silver halide emulsion layer or in a colloid layer contiguous therewith a phosphoric acid ester of a condensation product of an alkylene oxide with a butynediol.

PHOTOGRAPHIC ELEMENT CONTAINING A  
PHOSPHORIC ACID ESTER OF A BUTYNEDIOL-  
ALKYLENE

This invention relates to photographic emulsions and, more particularly, to the sensitization of these emulsions by incorporating therein certain phosphoric acid esters of polyoxyalkylene derivatives of butynediols.

Sensitization of silver halide emulsions by the use of polyoxyalkylene or polyalkylene oxides is well known and is described in U.S. Pat. Nos. 2,423,549 and 2,441,389 while the use of various derivatives of polyalkylene oxides as, for example, condensation products of an alkylene oxide with glycols is described in U.S. Pat. Nos. 2,240,472.

A deleterious effect with the use of these materials is their tendency to increase fog which is defined as the loss of sensitivity of the emulsion, during storage, resulting from the spontaneous occurrence of a developable species without exposure to light. Since the intensity of the resulting fog is dependent on both the inherent qualities of the emulsion and on the conditions of subsequent processing, the fog quantity becomes dependent, under constant conditions of development, on changes in such storage variables as time, temperature and relative humidity. Fog can also be the result of conditions present in high-temperature processing.

Since the addition of sensitizer compounds causes an increase in fog during storage, their use had been somewhat limited especially under the aforesaid conditions of high temperature and humidity storage or under conditions of high-temperature processing. This had led to the need for special and somewhat exotic antifogging compounds for use with these materials (see U.S. Pat. Nos. 2,704,716, 2,716,062 and 2,728,666). In a later development, described in U.S. Pat. No. 3,255,013, the use of certain polyoxyalkylene derivatives of butynediols was described in which conventional antifogging agents were suitable since these compounds did not cause an excessive increase in fog on storage.

It is an object of this invention, therefore, to provide novel sensitizers for silver halide emulsions.

It is a further object of this invention to provide such sensitizers which prevent formation or, at least, minimize fog development on storage and/or subsequent processing under conditions of high temperature.

It is also an object of this invention to provide such sensitizer compounds which reduce the development of surface static charges.

In accordance with this invention it has been found that certain phosphoric acid esters of the aforesaid polyoxyalkylene derivatives of a butynediol as hereinafter described either prevent formation of or substantially curtail fog development without any sacrifice of sensitivity. This is especially true where film is subject to storage and/or subsequent processing at high temperature.

Therefore this invention is based at least in part in the discovery that compounds of the phosphoric ester are satisfactory sensitizers for silver halide emulsions which do not cause excessive fog on development.

This invention is also based at least in part on the discovery that the incorporation of these compounds into silver halide emulsions results in increases in film speed (i.e., a marked increase in density for a given exposure) and improvement in the covering power of the developed silver. The covering power is defined as the ratio of the optical density at maximum density to the weight of silver per square decimeter in the developed image layer.

This invention is also based at least in part on the discovery that the incorporation of these compounds into silver halide emulsions results in a marked reduction in the development of surface static charge.

The phosphoric esters employed in photographic emulsions in accordance with this invention are compounds of the general formula:



wherein:

R is an alkylene group of from two to about four carbon atoms,

R<sub>1</sub>, R<sub>2</sub>, R<sub>3</sub> and R<sub>4</sub> are members selected from the group consisting of hydrogen and an alkyl group of from one to about five carbon atoms,

X is a member selected from the group consisting of hydrogen and the polyoxyalkylene derivative group said group being a compound having the general formula as set forth above



such that the compound can be either a mono-, di- or triester of phosphoric acid, or a mixture of the three, and m and n are positive integers such that the molecular weight of the ensuing compound is in excess of 300 and up to 150,000 or more.

The procedure below describes the preparation of a preferred phosphoric acid ester of a polyoxyalkylene derivative of butynediol.

Procedure A

Preparation of the phosphoric acid ester of the condensation product of ethylene oxide with 1,4-diisobutyl-1,4-dimethyl-butynediol.

Two hundred grams of a condensation product of ethylene oxide with 1,4-diisobutyl-1,4-dimethyl butynediol having a molecular weight of about 600 (and sold under the trademark Surfynol 465) were admixed at room temperature with 1 gram of hypophosphorous acid. Eleven grams of phosphorus pentoxide were added slowly over a 1-hour period within a temperature range of 25°-50° C. The system was then flushed with, and maintained under a blanket of, nitrogen, while the temperature was raised to 90°-95° C. After 4 hours, the system was cooled to 75° C., 2 grams of hydrogen peroxide (35 percent solution) were added and the temperature was again raised to 90°-95° C. for 15 minutes. The system was then cooled and the reaction product was decanted from the black residue. The product composition, a mixture of mono- and diester and nonionic material, was determined from Acid Number values. A typical product from a 4:1 mole ratio of surfactant to phosphorus pentoxide assays 34.8 percent monoester and 17.6 percent diester.

The aforesaid improvements can be realized by incorporating such phosphoric acid esters in the light-sensitive silver halide emulsion itself or in the undercoating, substratum, intermediate coating, overcoating or surface coating.

The phosphoric acid esters may also be advantageously employed in various types of photographic silver halide emulsions, e.g., nonsensitized emulsions, orthochromatic, panchromatic and X-ray emulsions. If used with sensitizing dyes, the ester material may be added to the emulsion before or after the dyes are added. Various silver halides may be used as the light-sensitive component, such as silver bromide, silver iodide, silver chloride or mixed silver halides. The phosphate esters may be used in emulsions intended for black-and-white photography or color photography, e.g., emulsions containing color-forming components. For the emulsion for color photography, a developer compound of the primary aromatic amine type as, for example, dimethyl aminoaniline should be incorporated with a suitable color-forming compound having a group such as hydroxyl or methylene to couple with the oxidizer group of the developer in the emulsion.

The dispersing agent in the photographic emulsion may be gelatin or some other hydrophilic compound, such as collodion, albumen, methyl cellulose, polyvinyl alcohol, polyvinylpyrrolidone or the like.

The quantity of the phosphate ester added to the emulsion will depend to a large extent on the layer into which it is incorporated. In any event, the concentration range, dependent on additive location, is from 0.5 to 15 grams per mole of silver halide.

Several examples are set forth below to illustrate the nature of the invention and the manner of carrying it out. However, the invention should not be considered as being limited to the details thereof.

### EXAMPLES 1-3

These examples illustrate the effectiveness of compounds of the type described above in increasing the speed of silver halide emulsions without any resultant increase in fog.

A gelatin-silver halide emulsion in which the silver halide consists of 4 percent silver iodide and 96 percent silver bromide was prepared in a conventional manner and brought up to its maximum light sensitivity. It was then readied for coating on film base, that is, melted at 40° C. and necessary coating finals were added as, for example, sensitizing dyes, antifogants, surfactants such as saponin and hardeners such as formaldehyde. A 10 percent aqueous solution of a phosphoric ester of a condensation product of ethylene oxide and 1,4-butyne diol having a molecular weight of about 500 was prepared and 10 cc. of this solution were added to a sample of the above-described emulsion, containing about 0.4 mol of silver halide. A sample of the same emulsion, but not containing the phosphoric acid ester, served as control. The so-prepared emulsion samples were coated on a suitable cellulose ester film base and dried. Samples of these film coatings were then exposed in a Type I-B Sensitometer and developed in a developer of the following composition:

|                                |            |
|--------------------------------|------------|
| Distilled water                | 500 ml.    |
| Metol                          | 2.2 grams  |
| Sodium sulfite, anhydrous      | 72.0 grams |
| Hydroquinone                   | 8.8 grams  |
| Sodium carbonate, monohydrated | 56.0 grams |
| Potassium bromide              | 14.0 grams |
| Water to make 1 liter.         |            |

The results are tabulated below:

| Example | Phosphoric acid ester, grams | Relative speed | Density <sup>2</sup> | Fog density <sup>3</sup> |
|---------|------------------------------|----------------|----------------------|--------------------------|
| 1-----  | 10                           | 100            | 0.18                 | 28                       |
| 2-----  | 1                            | 120            | 0.13                 | 29                       |
| 3-----  | 10                           | 130            | 0.12                 | 20                       |

<sup>1</sup> Control.

<sup>2</sup> After 6' dev.

<sup>3</sup> After 6 days oven test and 6' dev.

### EXAMPLES 4-7

These examples show that the addition of the type described in the examples above to emulsions containing compounds known to increase speed but also to increase fog density is effective in decreasing the resulting fog while having no deleterious effect on the speed.

The accelerator used was a lauryl ether of a polyethylene oxide with a molecular weight of approximately 350. It is sold under the trade mark BRIJ 35 (Atlas Power Co.). After drying, film samples were exposed and processed as described in Examples 1-3. The results are tabulated below:

| Example | Poly-<br>ethylene<br>oxide<br>lauryl<br>ether,<br>grams | Phos-<br>phoric<br>ester,<br>grams | Rel.<br>speed | Density <sup>2</sup> | Fog<br>density <sup>3</sup> |
|---------|---------------------------------------------------------|------------------------------------|---------------|----------------------|-----------------------------|
| 4-----  | 10                                                      | 0                                  | 100           | 0.18                 | 0.30                        |
| 5-----  | 1                                                       | -----                              | 140           | 0.30                 | 0.50                        |
| 6-----  | 1                                                       | 1                                  | 150           | 0.20                 | 0.34                        |
| 7-----  | 1                                                       | 10                                 | 160           | 0.16                 | 0.28                        |

<sup>1</sup> Control.

<sup>2</sup> After 6' dev.

<sup>3</sup> After 1 day at 140° F. and 50% R.H. and 6' dev.

### EXAMPLES 8-9

These examples illustrate the effectiveness of the phosphoric ester compounds when added to other than the emulsion layer.

A gelatin-silver halide emulsion in which the silver halide consists of 4 percent silver iodide and 96 percent silver bromide was prepared in a conventional manner. It was then readied for coating on film base, that is, melted at 40° C. and necessary coating finals were added such as sensitizing dyes, stabilizers and hardeners. The so-prepared emulsion samples were coated on a suitable cellulose ester base and dried. A 2 percent aqueous gelatin solution containing 6 percent (on weight of dry gelatin) of the phosphoric acid ester described above in examples 1-3 was coated on the emulsion side of the film base as an anti-abrasion layer. A sample of the same emulsion coated film base was also coated with an anti-abrasion layer consisting of a 2 percent aqueous gelatin solution without the phosphoric acid ester. After drying, the film samples were exposed and processed as described in examples 1-3 above. The results are tabulated below:

| Example | Anti-abrasion coating                                    | Relative speed | Density <sup>1</sup> | Fog density <sup>2</sup> |
|---------|----------------------------------------------------------|----------------|----------------------|--------------------------|
| 8-----  | 2% gelatin solution plus 0.12% of phosphoric acid ester. | 150            | 0.13                 | 0.20                     |
| 9-----  | 2% gelatin solution....                                  | 100            | 0.18                 | 0.30                     |

<sup>1</sup> After 6' dev.

<sup>2</sup> After 6 days oven test and 4' dev.

The data tabulated below list the results of measurements made on surface resistivity. Since these measurements are indicative of the static susceptibility of the film surface, they show the beneficial effect of the addition to the anti-abrasion coating of the compounds of this invention.

| Example | Anti-abrasion coating                            | Static susceptibility (surface resistivity $\times 10^3$ meg.) |                      |     |
|---------|--------------------------------------------------|----------------------------------------------------------------|----------------------|-----|
|         |                                                  | At 72° F. and 13% RH                                           |                      |     |
|         |                                                  | At 72° F. and 22% RH                                           | At 72° F. and 40% RH |     |
| 8-----  | 2% gelatin solution plus 0.12% phosphoric ester. | 180                                                            | 60                   | 10  |
| 9-----  | 2% gelatin solution....                          | 900                                                            | 900                  | 250 |

### EXAMPLES 10-12

These examples also illustrate the effectiveness of the phosphate ester compounds in reducing surface resistivity in noncurl emulsion formulations prepared in the conventional manner. Phosphate esters with the condensation products of ethylene oxide and 1,4-diisobutyl-1,4-dimethylbutylenediols in which the molecular weights were 500 (Surlynol 440) and 600 (Surlynol 465), respectively, were evaluated.

All samples contained 6 percent of the phosphate ester of a Surlynol (based on dry gelatin) and were conditioned for 12 hours at 72° F. and 50 percent relative humidity. Resistivity was determined using a Megohm Meter. The results are tabulated below.

| Example | Phosphate Ester Added           | Surface Resistivity (Meg.) |
|---------|---------------------------------|----------------------------|
| 10      | Control                         | $12 \times 10^4$           |
| 11      | Phosphate Ester of Surlynol 440 | $2.6 \times 10^4$          |
| 12      | Phosphate Ester of Surlynol 465 | $1.5 \times 10^4$          |

While exemplary embodiments of the invention have been described, the true scope of the invention is to be determined from the following claims.

75 What is claimed is:

1. A photographic element comprising a support and a light-sensitive silver halide emulsion layer having in a layer selected from the group consisting of the emulsion layer and a colloid layer contiguous therewith a phosphoric acid ester of a condensation product of an alkylene oxide having from two to four carbon atoms with a butynediol, said ester having a molecular weight of in excess of 300 and said ester being a compound of the following general formula:



wherein R is an alkylene group of from two to about four carbon atoms, R<sub>1</sub>, R<sub>2</sub>, R<sub>3</sub> and R<sub>4</sub> are members selected from the group consisting of hydrogen and an alkyl group of from one to about five carbon atoms, X is a member selected from the group consisting of hydrogen and the polyoxyalkylene derivative group as set forth in the general formula



and m and n are positive integers such that the molecular weight of the ensuing compound is in excess of 300 and up to 150,000 or more.

2. The photographic element as defined in claim 1 wherein the phosphoric ester is a compound having the following formula:



wherein m and n represent integers providing a molecular weight of at least 750, and X is a member selected from the group consisting of hydrogen and the polyoxyalkylene derivative group as set forth in the formula



15 3. The photographic element as defined in claim 2 wherein the phosphoric ester is the monoester.

20 4. The photographic element as defined in claim 2 wherein the phosphoric ester is the diester.

5. The photographic element as defined in claim 2 wherein the phosphoric ester is the triester.

25 6. The photographic element as defined in claim 2 wherein the phosphoric ester is a mixture of the mono-, di- and triesters.

7. The photographic element as defined in claim 1 wherein the phosphoric ester is located in the silver halide emulsion.

8. The photographic element as defined in claim 1 wherein the phosphoric ester is located in the surface coating layer.

30 9. The photographic element as defined in claim 1 wherein said phosphoric ester product is employed in an amount of from about 0.5 to 15 grams per mole of silver halide.

UNITED STATES PATENT OFFICE  
CERTIFICATE OF CORRECTION

Patent No. 3,615,612 Dated 10/26/71

Inventor(s) E. Scudder Mackey, Fritz Dersch, Fred S. Eiseman

It is certified that error appears in the above-identified patent and that said Letters Patent are hereby corrected as shown below:

In Title after "Butynediol-Alkylene" add  
--Oxide Condensate--.

Signed and sealed this 9th day of May 1972.

(SEAL)

Attest:

EDWARD M. FLETCHER, JR.  
Attesting Officer

ROBERT GOTTSCHALK  
Commissioner of Patents